

Aug. 3, 1954

P. PAWLYK

2,685,532

GAS PLATING WITH CHROMIUM HEXACARBONYL

Filed Oct. 8, 1951



INVENTOR  
PETER PAWLYK  
BY *P. Pawlyk*

ATTORNEYS

## UNITED STATES PATENT OFFICE

2,685,532

GAS PLATING WITH CHROMIUM  
HEXACARBONYLPeter Pawlyk, Dayton, Ohio, assignor to The  
Commonwealth Engineering Company of Ohio,  
Dayton, Ohio, a corporation of Ohio

Application October 8, 1951, Serial No. 250,304

18 Claims. (Cl. 117—50)

1

This invention relates to a process for the thermal decomposition of chromium hexacarbonyl to deposit metallic chromium on bases of metallic materials.

It is customary when attempting to use the metallic carbonyls as a source for the attainment of metal coatings to effect the decomposition of the carbonyl at relatively low pressures. This method of operation assists in the removal of the waste gases of decomposition, i. e. carbon monoxide from the plating area, permitting good contact between the metallic component of the carbonyl and the object to be plated. Particularly where the carbonyl employed has a relatively large proportion of non-metal to metal in the molecule, giving rise to very large volumes of waste gas, it has been considered necessary to operate at low pressures. Thus, for example, it has been customary to operate at pressures in the range of about 0.1 to 0.3 atmospheres where chromium hexacarbonyl is employed, since this compound gives rise to about six volumes of waste gas per molecular weight of metal deposited.

Operation at the low pressures has also been thought to be required in order to secure adherent metallic coats. At the lower pressures the mean free path of the molecules is considerably greater than at atmospheric pressure and the greater velocity attained by the molecules has been believed to be a requirement in the attainment of good bonding between the deposited metal and the base material.

This invention contemplates the provision of a unique process for the deposition of chromium plate from the vapors of chromium hexacarbonyl which process, due to the particular conditions of temperature and gas flow rates employed, is operable at atmospheric pressures. Thus the usual apparatus necessary for the maintenance of low pressures may be eliminated and the process effected with relatively simple equipment.

In the practice of the process of invention the chromium hexacarbonyl which vaporizes and decomposes at about 300° F. is maintained in solid form in a carburetor and contacted with an inert carrier gas, as carbon dioxide or nitrogen, at a temperature in the range of about 100 to 290° F. to secure a large vapor pressure of the carbonyl at a temperature below that of decomposition. The mixed vapors of carbonyl and carrier gas are then passed into a chamber, maintained at substantially atmospheric pressure, where the vapors contact the object to be plated and the temperature of which is above that at which decomposition of the carbonyl takes place, that

2

is, in the range of 550° to 700° F. The flow rate of the gases for successful plating is in the range of 1 to 3 liters per minute predicated on the flow of carrier gas to the carburetor and at substantially room temperature.

The invention will be more fully understood by reference to the following detailed description, examples, and drawings wherein the single figure illustrates apparatus useful in the process of invention:

Referring to the single figure of the drawing there is shown generally the major components of the gas plating system at A and B. The letter A indicates the source of plating vapors of controlled temperature, the letter B indicates the plating chamber system.

Referring to source A there is shown at 1 a tank or cylinder containing liquified carbon dioxide 2 under pressure. A valve 3 on the cylinder is adapted to control the flow of carbon dioxide vapor to conduit 5 through flow meter 4 secured in the line.

The remote end of conduit 5 is formed into a coil 6 which surrounds a carburetor 7 containing solid chromium hexacarbonyl 8. Coil 6 and carburetor 7 are immersed in oil 9 contained by tank 10 the assembly being heated by an electric heater 12. A thermostatic control having an element 13 immersed in oil 9 is connected by line 14 to heater 12 for temperature control of the oil in the known manner. A stirrer 15 operated by motor 16 through suitable belting 17 is used to prevent formation of localized temperature variations in the oil.

An insulated conduit 18 extends from the top of carburetor 7 and is connected through pump 19 at plating chamber system B at nozzle 20.

Plating chamber system B comprises a chamber 21 having an opening adapted to be closed by cover 22; workpiece 23 is suspended from a support 24 and is positioned between the nozzle 20 and a resistance heating element 25 supported on member 26 and electrically connected through connector 27 to a source of power (not shown).

The chamber is substantially surrounded with a water jacket having an inlet 29 and outlet 30. Also provided in a wall of the chamber and passing through the water jacket is an orifice 31 for the passage of waste gases from the chamber.

A conduit 32 secured in orifice 31 is provided with a trap 33 contained in a tank 34 surrounded with cooling water 35 which passes from inlet 36 through outlet 37. A line 38, open to the atmosphere, is provided to conduct away gases not subject to condensation in the trap.

In the process of invention the cleaned metal-

lic workpiece 23 is placed in the chamber and the system is first flushed free of air by passing an inert gas therethrough in any suitable manner.

The valve 3 on cylinder 2 is then opened to permit the passage of approximately 1½ liters per minute of carbon dioxide to the coil 6 contained in oil 9, the temperature of which has been raised to and is maintained at about 150° F. The carbon dioxide gas, heated to substantially the same temperature as the oil, then passes into carburetor 7.

Carburetor 7 and the solid carbonyl contents thereof have also been raised to about the temperature of the oil and consequently a considerable vapor pressure of the carbonyl exists in the chamber. The entering heated carbon dioxide under the influence of the pressures created by the material in tank 2 and the heat absorbed in coil 6, sweep the carbonyl vapors along to pump 19 and chamber 21.

The pump 19 may be utilized to supply sufficient energy to the plating gas to overcome losses occurring in line 18 or may serve to provide a definite velocity to the plating gas to achieve a desired result in the plating chamber.

The gases emanating from nozzle 20 fill chamber 21 and upon striking the workpiece 23, heated by means of elements 25, decompose to deposit metal on the workpiece. The plate surrounding element 25 may also receive a metallic deposit, but this is relatively unimportant as the same is heat conductive and recoverable. Substantially no deposition will take place on the chamber walls as they are cooled below metal decomposition temperature, i. e. to about 80° F. by the cooling water passing through jacket 28.

The relatively high, that is, substantially atmospheric pressure of the plating gases in chamber 21, when augmented by the pressures of the large volumes of waste gases, creates a flow to orifice 31, whereafter any undecomposed carbonyl plating gas is readily recovered in trap 33.

It may be noted that the expulsion of the waste gases is facilitated primarily by the inrush of plating gas and by the cooling effect of the walls remote from the workpiece which assist in the contraction of gas volume in their immediate vicinity, creating a pressure gradient towards the opening 9. Accordingly the gases move readily from the point of high pressure centrally of the chamber to the outlet and the plating action of the incoming gases is not impeded.

Specific examples of the conditions suitable for plating with chromium hexacarbonyl in the simplified apparatus set forth are given below:

#### Example I

|                                                     |                 |    |
|-----------------------------------------------------|-----------------|----|
| 1. Workpiece temperature (steel) _____ °F           | 600             | 60 |
| 2. Temperature of gas at carburetor _____ °F        | 240             | 60 |
| 3. Flow rate of carrier gas in liters per minute    | 1               |    |
| 4. Kind of carrier gas                              | CO <sub>2</sub> |    |
| 5. Time for deposition of .001" of chromium minutes | 15              | 65 |

#### Example II

|                                                     |                 |    |
|-----------------------------------------------------|-----------------|----|
| 1. Workpiece temperature (steel) _____ °F           | 600             | 70 |
| 2. Temperature of gas at carburetor _____ °F        | 180             | 70 |
| 3. Flow rate of carrier gas in liters per minute    | 1               |    |
| 4. Kind of carrier gas                              | CO <sub>2</sub> |    |
| 5. Time for deposition of .001" of chromium minutes | 20              | 75 |

#### Example III

|                                                     |                 |   |
|-----------------------------------------------------|-----------------|---|
| 1. Workpiece temperature (steel) _____ °F           | 700             | 1 |
| 2. Temperature of gas at carburetor _____ °F        | 280             |   |
| 3. Flow rate of carrier gas in liters per minute    | 1               |   |
| 4. Kind of carrier gas                              | CO <sub>2</sub> |   |
| 5. Time for deposition of .001" of chromium minutes | 6               |   |

#### Example IV

|                                                     |                 |   |
|-----------------------------------------------------|-----------------|---|
| 1. Workpiece temperature (steel) _____ °F           | 550             | 1 |
| 2. Temperature of gas at carburetor _____ °F        | 100             |   |
| 3. Flow rate of carrier gas in liters per minute    | 3               |   |
| 4. Kind of carrier gas                              | CO <sub>2</sub> |   |
| 5. Time for deposition of .001" of chromium minutes | 60              |   |

This example represents threshold conditions for the deposit of chromium.

#### Example V

|                                                                       |                 |   |
|-----------------------------------------------------------------------|-----------------|---|
| 1. Workpiece temperature (steel) _____ °F                             | 700             | 1 |
| 2. Temperature of gas at carburetor (carburetor temperature) _____ °F | 240             |   |
| 3. Flow rate of carrier gas in liters per minute                      | 1               |   |
| 4. Kind of carrier gas                                                | CO <sub>2</sub> |   |
| 5. Time for deposition of .001" of chromium minutes                   | 15              |   |

The metal upon which the deposition may take place is not a critical factor as cast iron as well as steel may be utilized and any metal which will withstand the required temperature and bond to the chromium is operable in the process of invention.

Other carrier gases which may be utilized include neon and argon as well as nitrogen and carbon dioxide.

The particular proportion of chromium hexacarbonyl present in the plating gas is not critical and may be varied to suit particular plating requirements and conditions of operation by varying the oil bath temperature and CO<sub>2</sub> flow. The time of plating will however be a function of the hexacarbonyl content and very dilute plating gases will require an excessively long period of operation for a given thickness of coating.

This application is related to co-pending applications Serial Nos. 250,301; 250,302; 250,303; 250,305; 250,306; and 250,307; all filed October 8, 1951, and all by the same inventor as the present application.

It will be understood that this invention is susceptible of modification in order to adopt it to different usages and conditions and accordingly it is desired to comprehend such modifications within this invention as may fall within the scope of the appended claims.

I claim:

1. A process of plating a metallic object with chromium comprising the steps of heating the object to be plated to a temperature above the decomposition point of gaseous chromium hexacarbonyl, and contacting the heated object with heat-vaporized flowing gaseous chromium hexacarbonyl in an atmosphere containing an inert carrier gas at substantially atmospheric pressures the temperature of the gases and the object being of such a nature that the hexacarbonyl decomposes to deposit metal on the object.

2. A process of plating a metallic object with chromium comprising the steps of heating the object to be plated to a temperature above the decomposition point of gaseous chromium hexa-

carbonyl, and contacting the heated object with heat-vaporized flowing gaseous chromium hexacarbonyl in an atmosphere containing an inert carrier gas at substantially atmospheric pressures the temperature of the gases and the object being such as to cause the hexacarbonyl to decompose and deposit metal on the object.

3. A process of plating a metallic object with chromium comprising the steps of heating the object to be plated to a temperature above the decomposition temperature of chromium hexacarbonyl, and contacting the heated object with heat-vaporized flowing gaseous chromium hexacarbonyl in an atmosphere containing carbon dioxide at substantially atmospheric pressures the temperature of the contacting gases being less than that of the decomposition point of the hexacarbonyl and the temperature of the object and gases and the flow rate being such that decomposition of the gases is caused to deposit metal on the object.

4. A process of plating a metallic object with chromium comprising the steps of heating the object to be plated to a temperature above the decomposition temperature of chromium hexacarbonyl, and contacting the heated object with heat-vaporized flowing gaseous chromium hexacarbonyl in an atmosphere containing nitrogen at substantially atmospheric pressures the temperature of the contacting gases being less than that of the decomposition point of the hexacarbonyl and the temperature of the object and gases and the flow rate being such that decomposition of the gases is caused to deposit metal on the object.

5. A process of plating a metallic object with chromium comprising the steps of heating the object to be plated to a temperature in the range of 550° to 700° F., and contacting the heated object with gaseous chromium hexacarbonyl at a flow rate of about 1-3 liters per minute in an atmosphere containing an inert carrier gas at substantially atmospheric pressure and a temperature range of about 100° to 290° F.

6. A process of plating a metallic object with chromium comprising the steps of heating the object to a temperature of about 600° F., vaporizing the chromium hexacarbonyl at a temperature of about 240° F., contacting the vaporized chromium compound with carbon dioxide gas at a temperature of about 240° F. and at a flow rate of about one liter per minute to form a mixture of the gases, and subjecting the heated object to the action of the flowing gases at substantially atmospheric pressure.

7. A process of plating a metallic object with chromium comprising the steps of heating the object to a temperature of about 600° F., vaporizing the chromium hexacarbonyl at a temperature of about 180° F., contacting the vaporized chromium compound with carbon dioxide gas at a temperature of about 180° F. and at a flow rate of about one liter per minute to form a mixture of the gases, and subjecting the heated object to the action of the flowing gases at substantially atmospheric pressure.

8. A process of plating a metallic object with chromium comprising the steps of heating the object to a temperature of about 700° F., vaporizing the chromium hexacarbonyl at a temperature of about 280° F., contacting the vaporized chromium compound with carbon dioxide gas at a temperature of about 280° F. and at a flow rate of about one liter per minute to form a mixture of the gases, and subjecting the heated object

to the action of the flowing gases at substantially atmospheric pressure.

9. A process of plating a metallic object with chromium comprising the steps of heating the object to a temperature of about 550° F., vaporizing the chromium hexacarbonyl at a temperature of about 100° F., contacting the vaporized chromium compound with carbon dioxide gas at a temperature of about 100° F. and at a flow rate of about 3 liters per minute to form a mixture of the gases, and subjecting the heated object to the action of the flowing gases at substantially atmospheric pressure.

10. A process of plating a metallic object with chromium comprising the steps of heating the object to be plated to a temperature of about 550-700° F., and contacting the heated object with vaporized hot gaseous chromium hexacarbonyl in an atmosphere of a carrier gas at substantially atmospheric pressure and carrier gas flow rates of one to three liters per minute the temperature of the gases being of such a nature that the hexacarbonyl decomposes to deposit metal upon the object.

11. A process of plating a metallic object with chromium comprising the steps of heating the object to be plated to a temperature of about 550-700° F., and contacting the heated object with vaporized hot gaseous chromium hexacarbonyl in an atmosphere of a carrier gas at substantially atmospheric pressure and carrier gas flow rates of one to three liters per minute, the temperature of the flowing carrier gas being less than the decomposition temperature of the chromium hexacarbonyl and greater than about 100° F.

12. A process of depositing approximately .001" of chromium on a metallic object comprising the steps of heating the object to be plated to a temperature in the range of about 550° F. to 700° F., and contacting the heated object with a mixture of the gases of chromium hexacarbonyl and carbon dioxide at a temperature in the range of about 100° F. to 290° F. at a flow rate of about one to three liters per minute and substantially atmospheric pressure for a period of about six to sixty minutes.

13. A process of depositing approximately .001" of chromium on a metallic object comprising the steps of heating the object to be plated to a temperature of about 600° F., and contacting the heated object with a mixture of the gases of chromium hexacarbonyl and carbon dioxide at a temperature of about 240° F. at a flow rate of about one liter per minute and substantially atmospheric pressure for a period of about 15 minutes.

14. A process of depositing approximately .001" of chromium on a metallic object comprising the steps of heating the object to be plated to a temperature of about 600° F., and contacting the heated object with a mixture of the gases of chromium hexacarbonyl and carbon dioxide at a temperature of about 180° F. at a flow rate of about one liter per minute and substantially atmospheric pressure for a period of about 15 minutes.

15. A process of depositing approximately .001" of chromium on a metallic object comprising the steps of heating the object to be plated to a temperature of about 700° F., and contacting the heated object with a mixture of the gases of chromium hexacarbonyl and carbon dioxide at a temperature of about 280° F. at a flow rate of about one liter per minute and substantially

atmospheric pressure for a period of about 15 minutes.

16. A process of depositing approximately .001" of chromium on a metallic object comprising the steps of heating the object to be plated to a temperature of about 550° F., and contacting the heated object with a mixture of the gases of chromium hexacarbonyl and carbon dioxide at a temperature of about 100° F. at a flow rate of about three liters per minute and substantially atmospheric pressure for a period of about 15 minutes.

17. A process of plating a metallic object with chromium comprising the steps of heating the object to be plated to a temperature of about 700° F., vaporizing the chromium hexacarbonyl at a temperature of about 240° F., contacting the vaporized chromium compound with carbon dioxide gas at a flow rate of about one liter per minute to form a mixture of the gases, and subjecting the heated object to the action of the flowing gases at substantially atmospheric pressure.

18. A process of depositing approximately .001" of chromium on a metallic object comprising the

steps of heating the object to a temperature of about 700° F., vaporizing the chromium hexacarbonyl at a temperature of about 240° F., contacting the vaporized chromium compound with carbon dioxide gas at a flow rate of about one liter per minute to form a mixture of the gases, and subjecting the heated object to the action of the flowing gases for a period of about 15 minutes at substantially atmospheric pressure.

10 References Cited in the file of this patent

UNITED STATES PATENTS

| Number    | Name     | Date          |
|-----------|----------|---------------|
| 2,063,596 | Feiler   | Dec. 8, 1936  |
| 2,344,138 | Drummond | Mar. 14, 1944 |
| 2,475,601 | Fink     | July 12, 1949 |

OTHER REFERENCES

Plating Molybdenum, Tungsten, and Chromium by Thermal Decomposition of their Carbonyls, J. J. Lander and L. H. Garmer, American Institute of Mining and Metallurgical Engineers, Technical Publication #2259, September 1947, page 3.